# EUROPEAN PATENT SPECIFICATION

(11) **EP 0 242 283 B1**
(45) Date of publication and mention of the grant of the patent: **07.11.1990**
(21) Application number: 87400808.9
(22) Date of filing: 09.04.1987
(51) Int. Cl.: C22C 38/14, H01F 1/08

(54) **A rare earth-based alloy for permanent magnet**
Legierung auf Basis seltener Erden für Permanentmagnet
Alliage à base de terres rares pour aimant permanent

(30) Priority: 12.04.1986 JP 84723/86; 12.04.1986 JP 84724/86
(43) Date of publication of application: 21.10.1987
(73) Proprietor: Shin-Etsu Chemical Co., Ltd., Chiyoda-ku Tokyo 100 (JP)
(72) Inventor: Ohashi, Ken, Takefu-shi Fukui-ken (JP); Yokoyama, Toshikazu, Fukui-shi Fukui-ken (JP); Tawara, Yoshio, Fukui-shi Fukui-ken (JP)
(74) Representative: Armengaud Ainé, Alain

(56) References cited:
- US-A- 4 221 613
- Ullmanns Encyklopädie der technischen Chemie, 4, Band 21, S. 236
- Webster's Third New International Dictionary

## Description

### BACKGROUND OF THE INVENTION

The present invention relates to a rare earth-based alloy for permanent magnet having excellent magnetic properties and suitable as a component of various kinds of electric and electronic instruments.

Various kinds of rare earth-based permanent magnet alloys have been developed hitherto and are under production in large quantities including the samarium-cobalt magnet alloys of the chemical composition SmCoₛ. The magnetic properties of the permanent magnets of this type are so excellent that the maximum energy product (BH)max thereof exceeds 20 MGOe in the magnets manufactured under experimental conditions or is constantly in the range from 16 to 18 MGOe in the magnets manufactured as industrial products. Accordingly, these permanent magnets are widely used in a variety of applications such as speakers, electric motors, metering instruments and the like in which the permanent magnets are required to exhibit high performance. One of the problems in the samarium-based permanent magnets is the high production costs as a consequence of the high content of relatively expensive cobalt metal therein up to 60% by weight or more. It would therefore be a desirable measure to replace the cobalt metal with a less expensive metal such as iron and some attempts have been made hitherto in this direction. No fruitful results, however, have yet been obtained in such an attempt presumably due to the absence of possible solid-solution formation of iron with the SmCo₅ intermetallic compound.

On the other hand, several binary intermetallic compounds of rare earths and iron are known including the compounds of the formulas RFe₂, RFe₃ and R2Fen, R being a rare earth element. These rare earth-iron intermetallic compounds, however, are not utilized as a permanent magnet due to the low value of either one of the magnetic parameters of Curie point T_{c}, saturation magnetization 4nMₛ and crystalline magnetic anisotropy constant Kᵤ, In contrast to the series of rare earth-cobalt intermetallic compounds including the RCos-type compounds having the crystalline structure of CaCus, of which the above mentioned SmCo₅ alloy is practically utilized as a material of permanent magnets, no RFeₛ type compounds were known for long in the series of rare earth-iron compounds, at least, in the form of a bulk body. It was only in 1984 that Cadieu, et al. reported in Journal of Applied Physics, volume 55, page 2611 (1984) that thin films of SmFes and (SmTi)ₓFE₁oo-_{x'} in which the atomic ratio of Ti:Fe was 1:9 or 1:19, could be formed by the method of sputtering. These intermetallic compounds in the form of a thin film reportedly have a hexagonal crystalline structure of CaCus. These thin films formed by the sputtering method, however, were in the state of a metastable phase and it was generally understood that such an intermetallic compound could not exist as a bulk body. Therefore, the only permanent magnet based on a rare earth-iron binary compound so far reported is the magnet in a metastable phase prepared by the quenched thin-film method disclosed by Croat, et al. in IEEE Transactions on Magnetics, volume MAG 18, page 1442 (November, 1982). The quenched thin-film magnet prepared by this method is isotropic and based on a metastable phase so that the magnet is not free from the problem of low stability so that the magnets of this type are not in practical use.

Turning now to the recently highlighted neodymium-iron-boron magnets formed of a ternary compound of a chemical composition of the formula R₂F₁₄B, they are promising as a high-performance permanent magnet since the base components are inexpensive neodymium and iron and the magnetic properties thereof are even better than those of the samarium-cobalt magnets. These neodymium-iron-boron magnets are, however, not free from a very serious problem that they are highly susceptible to rusting so that the magnets cannot be used practically without providing a protective coating. This disadvantage can hardly be overcome and no practical solution of the problem has yet been obtained to give a possibility of industrial production of the magnets of this type.

### SUMMARY OF THE INVENTION

An object of the present invention is therefore to provide a rare earth-based permanent magnet having magnetic properties equivalent to or even better than those of the samarium-cobalt permanent magnets without using or by decreasing the amount of expensive cobalt as well as to provide a rare earth-based alloy as a base material of such a permanent magnet.

Thus, the permanent magnet alloy of the present invention consists of:
(a) form 12 to 45% by weight of a rare earth element or a combination of rare earth elements;
(b) from 0.1 to 10% by weight of titanium; and
(c) the balance of iron or a combination of iron and cobalt, the amount of iron being at least 40% by weight thereof, including unavoidable impurities.

Further, the permanent magnet of the invention is a sintered body of a powder of the above defined rare earth-based alloy having magnetic anisotropy.

### BRIEF DESCRIPTION OF THE DRAWING

FIGURE 1 is a graph showing the magnetization of inventive and conventional samarium-based alloys as a function of temperature.
FIGURE 2 illustrates the X-ray diffraction diagrams of the same alloys using CuKa line.

### DETAILED DESCRIPTION OF THE PREFERRED EMBODIMENTS

In respect of the problem of possible existence of RFes phase, the results of experiments hitherto undertaken support that no such a 1:5 phase or, in particular, SmFe₅ phase is formed even when samarium and iron are melted together and alloyed in a proportion corresponding to the composition of SmFeₛ although three phases of SmzFen, SmFe₂ and SmFe₃ could be found as is indicated by the results obtained in the measurement with a vibration magnetometer and in the X-ray diffractometry as is shown in FIGURES 1 and 2.

With an object to obtain a rare earth-iron based permanent magnet having excellent magnetic properties equivalent to those of the imaginary SmFeₛ magnet, the inventors have conducted extensive investigations on a third additive element to be added to the rare earth-iron binary magnet alloys and arrived at discoveries that addition of titanium would give a quite satisfactory result and a hitherto unknown ternary intermetallic compound of samarium, titanium and iron can exist in a bulky form by the optimization of the amount of substitution of titanium for the rare earth element or, in particular, samarium. Thus, a ternary alloy of samarium, titanium and iron was prepared in such a proportion as to correspond to the formula of SmTiFeio and the alloy was subjected to the measurement of the magnetization as a function of temperature and X-ray diffractometry to give the results shown in FIGURES 1 and 2, respectively. These figures indicate that, in clear difference from those of the SmCos-type crystalline structure, crystallographic indices approximately corresponding to those of the tetragonal crystalline structure can be allotted to the peaks in the X-ray diffractometric diagram of the ternary ally and the temperature dependency of the magnetization thereof is also close to that of a single-phase alloy leading to a conclusion that the ternary compound of samarium, titanium and iron is imparted with stability as a result of introduction of titanium into the samarium-iron binary alloy. The further continued investigations have led to confirmation that the above described unique phenomenon is held also for the rare earth elements in general other than samarium including yttrium.

Thus, the present invention provides, as an embodiment, a ternary alloy composed of (a) from 12 to 45% by weight of a rare earth element or a combination of rare earth elements; (b) from 0.1 to 10% by wieght of titanium; and (c) the balance of iron including unavoidable impurities. Namely, the magnet alloy can be obtained by melting the component metals together and the alloy is finely pulverized followed by the powder metallurgical processing of the powder by compression molding and sintering. When the amount of the rare earth component in the alloy formulation is outside the above specified range, the ternary compound would be less stable and, therefore, any amounts thereof smaller than 12% by weight and larger than 45% may result in a disadvantageously rapid decrease in the coercive force iH_{c} and saturation magnetization 4nMₛ, respectively. The above mentioned range for titanium is also critical because the ternary compound is less stable when the amount of titanium is smaller than 0.1% by weight while the fraction of the phase of the ternary compound is decreased when the amount of titanium is larger than 10% by weight. The rare earth element here implied include the so-called lanthanoid elements having atomic munbers of 57 to 71 and yttrium. Any of these rare earth elements can be used either singly or as a combination of two kinds or more according to need.

The rare earth-based permanent magnet of the invention prepared of the ternary alloy contains the stable phase of the ternary compound as a result of the introduction of titanium so that the Curie point thereof is about 310_{°}C when the rare earth element is samarium which is much higher than 120°C of the Sm₂Fe₁₇ phase. In addition, the saturation magnetization is also greatly increased so that the thus obtained permanent magnet has very high magnetic properties. Moreover, the rare earth-titanium-iron permanent magnet of the invention can be imparted with magnetic anistropy by the powder metallurgical method so that the overall magnetic performance of the inventive permanent magnet can be almost equivalent to or even better than the samarium-cobalt based magnets.

Despite the high content of iron in the alloy of the inventive permanent magnet, which is formed mainly of a tetragonally crystalline phase, the inventive permanent mgnet is highly corrosion-resistant and free from rusting in clear contrast to the neodymium-iron based magnets. Accordingly, the inventive permanent magnets can be used in practical applications without any prtective coating on the surface although the corrosion resistance thereof can of course be further increased by a protective coating or surface treatment by forming a resinous layer or a metallic layer formed by electrolytic or electroless plating, vacuum vapor deposition, sputtering or ion plating.

Further, the ternary alloy can be processed into a thin film having a high coerqive force by the quenched thin-film method and the thin film can be finely pulverized into fine particles of which magnetically isotropic permanent magnets can be prepared. It is of course that the magnetically anisotropic sintered magnet is pulverized into fine particles of which anisotropic plastic magnets can be prepared.

As is mentioned above, the permanent magnet of the ternary alloy of samarium, titanium and iron has a Curie point of about 310°G. Although this Curie point is well within the practically acceptable range, it is of course desirable to have a higher Curie point when comparison is made with the SmCos permanent magnets having a Curie point at about 740_{°}C. In this regard, the inventors have further continued extensive investigations and arrived at a discovery that a magnetic alloy suitable for the purpose can be obtained when a solid solution is formed of the above described ternary compound of rare earth, titanium and iron with cobalt. For example, an increase by about 40 to 100°C can be obtained in the Curie point of the ternary alloy when 10 atomic % of iron in the alloy is replaced with cobalt although the increment depends on the kind of the rare earth element. The Curie point T_{c} is increased approximately linearly with the increase in the amount of replacement of iron with cobalt up to 50% replacement by weight but thereafter the increment in the Curie point is relatively small with further increased replacement of iron with cobalt to finally level off. In addition, the saturation magnetization of the magnet is increased as a trend though dependent on the kind of the rare earth element by the substitution of cobalt for a part of iron in the ternary magnet alloy of rare earth, titanium and iron to level off with increase of the proportion of cobalt relative to iron.

It should be noted, however, that replacement of iron with cobalt has some adverse effect of decreasing the coercive force of the magnet. For example, more than 40% replacement of iron with cobalt is undesirable due to the great decrease in the coercive force of the magnet. This is the reason for the limitation that more than 60% by weight or, preferably, more than 40% by weight of iron should not be replaced with cobalt.

In the following, the rare earth-based alloy for permanent magnets and the sintered permanent magnet of the alloy accor ing to the invention are described in more detail by way of examples.

### Example 1.

Metals of samarium, titanium and iron each having a purity of 99.9% were taken by weighing in the proportion indicated in Table 1 below and melted together in a high-frequency induction furnace. The melt was cast into a water-cooled, copper-made casting mold to form an ingot of the alloy. The ingot was crushed and then pulverized in a jet mill using nitrogen gas as the ject gas to give a fine powder having an average particle diameter in the range from 2 to 10 µm. The powder was compression-molded under a pressure of 1.5 tons/cm² with the particles oriented in a static magnetic field of 15 KOe into a green body, which was sintered by heating in an atmosphere of argon gas for 1 hour at a temperature in the range form 1000 to 1200 _{°}C and then subjected to thermal aging for 4 hours at a temperature in the range from 500 to 900 _{°}C followed by quenching.

The thus obtained magnetically anisotropic sintered body after the thermal aging was subjected to the measurement of the density of residual magnetic flux Bᵣ, coercive force iH_{c} and maximum energy product (BH)ₘₐₓ to give the results shown in Table 1 for the three different formulations of the alloys No. 1, No. 2 and No. 3. For comparison, Table 1 also includes the results of the magnetic measurement of a sintered body of a samarium-iron al loy corresponding to SmFeₛ (No. 4) prepared in the same manner as above. As is shown in the table, this comparative sintered body had only negligibly small values of coercive force and maximum energy product.

### Example 2.

Metals of praseodymium, samarium, cerium, titanium and iron were taken by weighing in the proportion indicated in Table 2 and magnetically anisotropic sintered bodies were prepared each in the same manner as in Example 1. The coercive force iH_{c} of these sintered bodies was measured to give the results shown in the table which supports the conclusion that the coercive force is little affected by the replacement of samarium with other rare earth elements.

### Example 3.

Magnetically anisotropic sintered permanent magnets No. 1 to No. 4 were prepared each in the same manner as in Example 1 except that the magnetic alloy was prepared from metals of neodymium, titanium, iron and cobalt each having a purity of 99.9% taken by weighing in the proportion indicated in Table 3.

These sintered permanent magnets were subjected to the measurement of the density of residual magnetic flux Br, coercive force iH_{c} and maximum energy product (BH)max as well as Curie point to give the results shown in the table, in which △T_{c} means the increment of the Curie point T_{c} in _{°}C obtained by the replacement of a part of iron with cobalt.

### Example 4.

Magnetically anisotropic sintered permanent magnets No. 1 and No. 2 were prepared in the same manner as in the preceding examples from metals of samarium, cerium, titanium, iron and cobalt taken by weighing in the proportion indicated in Table 4 below. These sintered permanent magnets were subjected to the measurement of the magnetic properties to give the results shown in the table.

## Claims

1. A rare earth-based alloy for permanent magnet consisting of:
(a) from 12 to 45% by weight of a rare earth element or a combination of rare earth elements;
(b) from 0.1 to 10% by weight of titanium; and
(c) the balance of iron or a combination of iron and cobalt, the amount of iron being at least 60% by weight thereof, including unavoidable impurities.

2. The rare earth-based alloy for permanent magnet as claimed in claim 1 wherein the rare earth element is selected from the group consisting of the elements of the atomic number of from 57 to 71 and yttrium.

3. A permanent magnet which is a sintered body of a powder of a rare earth-based alloy consisting of:
(a) from 12 to 45% by weight of a rare earth element or a combination of rare earth elements;
(b) from 0.1 to 10% by weight of titanium; and
(c) the balance of iron or a combination of iron and cobalt, the amount of iron being at least 60% by weight thereof, including unavoidable impurities.

## Patentansprüche

1. Legierung auf der Basis seltener Erden für Permanentmagnete bestehend aus:
(a) 12 bis 45 Gew.-% eines Elementes seltener Erden oder einer Kombination von Elementen seltener Erden;
(b) 0,1 bis 10 Gew.-% Titan; und
(c) in der Menge der Differenz bis 100% aus Eisen oder einer Kombination aus Eisen und Kobalt, wobei deren Eisenanteil mindestens 60 Gew.-% beträgt, einschließlich unvermeidbarer Verunreinigungen.

2. Legierung auf der Basis seltener Erden für Permanentmagnete nach Anspruch 1, wobei das Element seltener Erden zur Gruppe aus Elementen mit der Ordnungszahl von 57 bis 71 sowie Yttrium gehört.

3. Permanentmagnet in Form eines Sinter-Körpers aus einem Pulver einer Legierung auf der Basis seltener Erden bestehend aus:
(a) 12 bis 45 Gew.-% eines Elementes seltener Erden oder einer Kombination von Elementen seltener Erden;
(b) 0,1 bis 10 Gew.-% Titan; und
(c) in der Menge der Differenz bis 100% aus Eisen oder einer Kombination aus Eisen und Kobalt, wobei deren Eisenanteil mindestens 60 Gew.-% beträgt, einschließlich unvermeidbarer Verunreinigungen.

## Revendications

1. Alliage à base de terres rares pour aimant permanent, constitué de:
(a) 12 à 45% en poids d'un élément des terres rares, ou d'une combinaison d'éléments des terres rares;
(b) 0,1 à 10% en poids de titane; et
(c) le reste étant du fer ou une combinaison de fer et de cobalt, la proportion en fer étant d'au moins 60% en poids, y compris les impuretés inévitables.

2. Alliage à base de terres rares pour aimant permanent, selon la revendication 1, dans lequel l'élément des terres rares est choisi dans le groupe constitué des éléments dont les numéros atomiques sont compris entre 57 et 71, et l'yttrium.

3. Aimant permanent qui est un corps fritté formé d'une poudre d'un alliage à base de terres rares, constitué de:
(a) 12 à 45% en poids d'un élément des terres rares, ou d'une combinaison d'éléments des terres rares;
(b) 0,1 à 10% en poids de titane; et
(c) le reste étant du fer ou une combinaison de fer et de cobalt, la proportion en fer étant d'au moins 60% en poids, y compris les impuretés inévitables.
